

Patented Oct. 30, 1923.

1,472,691

## UNITED STATES PATENT OFFICE.

WALTER O. SNELLING, OF ALLENtown, PENNSYLVANIA, ASSIGNOR TO TROJAN POWDER COMPANY, OF NEW YORK, N. Y., A CORPORATION OF NEW YORK.

### NITROSTARCH EXPLOSIVE.

No Drawing.

Application filed October 14, 1922. Serial No. 594,592.

To all whom it may concern:

Be it known that I, WALTER O. SNELLING, a citizen of the United States, residing in Allentown, Lehigh County, Pennsylvania, 5 have invented a Nitrostarch Explosive, of which the following is a specification.

My invention relates to nitrostarch explosives, and more particularly to the preparation of nitrostarch explosives of 10 exceptional strength and brisance.

It has long been known that explosives possessing desirable properties could be made by mixing together nitrostarch and an inorganic nitrate of high oxygen value 15 such as the nitrates of sodium, potassium, and ammonium, and explosives consisting of mechanical mixtures of nitrates of ammonium and sodium with nitrostarch have long been used as commercial explosives. In general, the higher the oxygen value of a nitrate, the better its behavior as a component of an explosive mixture.

I have discovered that when nitrostarch is mixed with nitrate of lead, explosives 25 possessing exceptional characteristics are obtained in spite of the fact that the oxygen content of lead nitrate is comparatively low. Thus while sodium nitrate contains 56.5% of oxygen, while lead nitrate contains but 30 29%, I find that the strength of an explosive containing lead nitrate is materially greater than the strength of an explosive containing an equivalent weight of sodium nitrate. Comparative tests of a considerable number 35 of explosives containing corresponding quantities of sodium nitrate and lead nitrate have invariably shown that the explosives containing lead nitrate possess greater greater strength than explosives containing 40 sodium nitrate, instead of possessing less strength as would be expected from the smaller amount of available oxygen contained in lead nitrate as compared with the amount of oxygen available in sodium 45 nitrate.

As an example of an explosive made in accordance with my present invention, I may take thirty parts of nitrostarch, sixty-

nine and five-tenths parts of lead nitrate, and one-half of one part of oil. The three 50 constituents are thoroughly mixed together, and may then be packed in cartridges in the usual way. The explosive so prepared possesses exceptional strength and forms a very desirable explosive for commercial 55 blasting where maximum shattering effect is desired.

By increasing the amount of oil slightly, a reduction in sensitiveness of the explosive is obtained without any corresponding 60 reduction in its strength when detonated by a suitable priming charge. For explosives for filling shells or for other purposes where a relatively insensitive explosive of great strength is required, I prefer to 65 employ a mixture containing 40% of nitrostarch, 57% of lead nitrate, and 3% of oil.

It will be evident that I may employ any of the other ingredients commonly employed in explosives, in connection with the compositions embodying my present invention. 70 I may, for example, add an anti-acid such as sodium bicarbonate or zinc oxide for the purpose of increasing the stability of my explosive, or I may add any organic 75 stabilizer such as diphenylamine or urea. I may substitute for a part of my lead nitrate a cheaper nitrate such as sodium nitrate for the purpose of reducing the cost of my finished product. I may add a 80 combustible ingredients such as wood pulp, or flour, or I may add a material such as sulfur that can combine with the lead set free by the explosion of my compound, and in general I may modify my explosive mixtures in accordance with any of the well 85 known methods of the art.

I claim:

1. An explosive comprising nitrostarch and lead nitrate. 90
2. A nitrostarch explosive containing as a constituent lead nitrate.
3. An explosive comprising nitrostarch, lead nitrate, and an oil.

WALTER O. SNELLING.